

G. R. MEYERCORD.

PROCESS OF MAKING HEAVY STRUCTURAL WHITE GLASS.

APPLICATION FILED MAR. 4, 1912.

1,108,205.

Patented Aug. 25, 1914.



Fig. 1.



Fig. 2.

WITNESSES:

Frank L. Stubbs

R. A. Saegg

INVENTOR

George R. Meyercord

By Chamberlin & Prendergast  
Atty.

# UNITED STATES PATENT OFFICE.

GEORGE R. MEYERCORD, OF CHICAGO, ILLINOIS.

## PROCESS OF MAKING HEAVY STRUCTURAL WHITE GLASS.

1,108,205.

Specification of Letters Patent. Patented Aug. 25, 1914.

Application filed March 4, 1912. Serial No. 681,357.

To all whom it may concern:

Be it known that I, GEORGE R. MEYERCORD, a citizen of the United States, residing at Chicago, county of Cook, State of Illinois,

5 have invented a certain new and useful Improvement in Processes of Making Heavy Structural White Glass, and declare the following to be a full, clear, and exact description of the same, such as will enable 10 others skilled in the art to which it pertains to make and use the same, reference being had to the accompanying drawings, which form a part of this specification.

My invention relates to the art of making 15 thick slabs or sheets of glass, particularly white glass, for structural purposes; and, generally speaking, it has for its objects to improve the quality of the product, cheapen the cost, and reduce the size of plant necessary for manufacturing slabs or sheets ranging from the thinnest to the thickest.

A good uniform quality of white glass in sheets or slabs of the thickness of ordinary transparent plate glass may be cast, rolled 25 and annealed economically in substantially the same way as plate glass; but where a thickness of an inch or more is required, as for tops of counters or tables, partitions, or the like, problems in manufacturing 30 are encountered which have heretofore militated against quality and uniformity of product, economy of manufacture, and a low initial cost of plant for producing both thick and thin slabs or sheets.

35 Thus a thick slab or sheet of considerable size requires more material than can be dipped out of a supply of molten glass by the ordinary ladle of maximum capacity, and therefore recourse has been had to pots,

40 in each of which is mixed a charge sufficient to form a single slab or sheet. This makes it necessary to provide both pots and ladles where both thick and thin sheets are to be made, and increases the cost of the plant

45 above that which would be necessary if only ladles were required for all kinds of sheets. Another disadvantage is that the quality of

50 the product, as to coloring and otherwise, cannot be kept as uniform where many individual charges or small masses are prepared separately, as in the potting method, as where a much larger mass is prepared and then divided into units, as in the ladling method; and consequently it has heretofore

55 been impossible to secure the same uniformity in a quantity of thick sheets as in the

case of thin sheets. Again, it is difficult to cast and roll a perfect thick sheet in the old way, and the waste increases rapidly with the thickness.

60 After the sheet has been formed it must be annealed, this being accomplished, in the case of thin sheets, in ordinary annealing furnaces or leers. However, it has been found to be impracticable to anneal thick 65 sheets made in the old way in such leers, on account of the great length of time the sheets were required to remain in the leers to effect the annealing; and consequently it has been the practice to provide closed chambers on the order of large Dutch ovens, in which the sheets may remain for days in order to become annealed. It will thus be seen that, by reason of the slowness of the annealing process, numerous ovens, covering 70 a large space, are required if the output is to be considerable. Here, again, is a duplication of apparatus where both thick and thin 75 sheets are manufactured, due to the difference in the character of the annealing processes. Even though there has been a departure in the manufacture of thick sheets from the process of making thin sheets, and even though especial apparatus has been 80 provided, this has not resulted in a product 85 as uniform as the thin sheets and, because the thickness of the sheets has prevented such a readjustment of the structure of the glass to make the texture fine and even, the quality of the thick sheets, structurally considered, has been inferior to that of the thin 90 sheets. This is evidenced by the fact that it has heretofore been deemed necessary to chisel a sheet in order to divide it, instead of cutting it like ordinary glass.

95 My invention is intended to overcome the difficulties heretofore noted, to make possible the use of the same apparatus for manufacturing sheets of any desired thickness, to insure uniformity of product, and to secure 100 strength and fineness in heavy sheets.

The various features of novelty whereby my invention is characterized will herein-after be pointed out with particularity in the claims; but for a full understanding of 105 my invention and of its objects and advantages reference may be had to the following detailed description, taken in connection with the accompanying drawing, wherein:

110 Figure 1 is a side view of a simple form of apparatus for carrying out my invention.

and Fig. 2 is a side elevation of a portion of a machine arranged to secure one of the advantages of the principal invention.

I have discovered that the solution of the whole problem of producing thick white-glass sheets is solved by making them in layers, fused together in the rolling process, or, in other words, by making each sheet of laminae merged into each other to form a unitary structure. I accomplish this by beginning a layer whose thickness is one-half, one-third, one-fourth, one-fifth, or any other fraction of that of the finished sheet, casting upon this a second layer, then a third, and so on until the desired thickness is obtained. Each layer is formed progressively as are the sheets in the ordinary plate-glass art and, as it grows, it is merged into the superposed layer, so that the finished sheet is made up of a number of united layers, each of which has had the entire surface of at least one face exposed at some time during the process. Thus the gases are allowed to escape at the surface of each layer during the forming process instead of from the single upper surface as in the old process; each layer is toughened substantially as if it were an independent unit; and a cooling action occurs throughout the entire mass instead of only at the surfaces of the thick sheet. Consequently the sheet, when completed, is more uniform in texture, and is tougher and stronger than a sheet of similar thickness when rolled as a single layer. Furthermore, there is not the great difference in temperature between the middle of the sheet and the exposed faces that exists in the thick sheet formed in the old way. The result of this is that the thick sheets can be annealed effectively and rapidly by passing them through the usual leers employed for annealing ordinary thin sheets. It will thus be seen that a large output of thick sheets may be obtained without having capital invested in numerous annealing ovens of the old type, without having a large inactive stock housed in the ovens, and without making it necessary to have separate annealing plants for thick sheets and thin sheets. It will also be evident from the foregoing that the molten mass may be prepared in the same way and handled in the same way in the production of thick sheets as in the production of thin sheets. If the thick sheet is made of two layers, then only one-half of the total material is required for each layer and the amount may be handled in one of the usual ladles which might not, however, be large enough to contain the material for a whole sheet. For heavier sheets three or more layers may be employed, the material for the several layers being supplied by separate ladles. Therefore it is possible to prepare the mixture in large quantities, dipping it

out with the usual ladles, not only for one sheet but for a large number; thus insuring greater uniformity of product than is possible where the material for each sheet must be mixed in a pot because the quantity is greater than a single ladle will hold. Thus it will be seen that by my method of making sheets of an inch or more in thickness a superior product is obtained at a low cost and without requiring separate plants for thick and thin sheets. Furthermore, the sheets can be cut like ordinary thin sheets, making chiseling unnecessary.

In Fig. 1 of the accompanying drawing I have illustrated diagrammatically the preferred method of carrying out the principal step of my invention. Referring to this figure, 1 represents a suitable table of any usual construction; and 2, 3 and 4 represent parallel rolls extending transversely of the table and separated from each other lengthwise of the table. Where there are three rolls, as shown, the first, roll 2, will lie above the table a distance about one-third of the thickness of the sheet to be cast; the second roll, 3, will be farther away from the table; and the last roll, 4, will be spaced from the table the proper distance to give the desired thickness to the sheet. The rolls and the table may be operated in any suitable or usual way. The first ladle is emptied in front of the roll 2, leaving a molten mass 5 to be pressed between the roll and the table into a layer 6. The second ladle is emptied in front of the roll 3 on top of the layer 6, providing a second heap, 7, to be rolled into a layer, 8, superimposed upon and merged with the underlying layer. It will be seen that the first layer has its upper face exposed behind the first roll so that the gases are free to pass off and a partial cooling of the layer takes place. The molten mass in front of the second roll causes the partial skin on the under layer to fuse so as to produce a complete union between the first two layers; but the heating of the one layer is accomplished by a cooling of the overlying layer and therefore the center of the mass as it passes under the second roll is much cooler than it would be in a single layer having the thickness of the two layers combined. Similarly the third ladle is emptied in front of the third roll, 4, and the heap 9 is rolled into a layer, 10, on top of the two layers previously formed; the upper surface of layer 8 having been partially cooled and being again fused by the hot overlying material. The layers 8 and 10 are fused together and leave a second partially-cooled stratum in the finished sheet. Thus the material of the sheet has been worked over three times when it passes under the last roll and has been toughened and has been partially cooled in the interior thereof, so that, upon cooling, it is not subjected to the enormous strains

- which are imposed on a sheet of the same thickness rolled as a single layer and having its center at almost the same temperature as when first poured. Furthermore, the upper 5 surface of the sheet is smoother and more finished than in the case of a sheet having only a single rolling. While I have illustrated three rolls, I do not confine myself to any particular number.
- 10 It will be seen that the finishing of the surface of glass sheets by means of successive rollings is not necessarily confined to thick sheets made in layers; but is applicable to cast sheets of any thickness and of one or 15 more layers. Thus in Fig. 2 I have illustrated an arrangement in which two rolls, 11 and 12, are spaced at equal distances from the table 13, the first roll forming the sheet 14 and the other roll following and finishing 20 the surface.
- I claim:
1. The method of making sheets or slabs of glass having a thickness of one inch or more, which consists in making them in 25 layers formed progressively and fused together as they are formed.
  2. The method of making sheets or slabs of glass having a thickness of one inch or more, which consists in casting and rolling a plurality of superimposed layers in such 30 a manner that as each layer is formed the succeeding layer is applied and fuses the partially formed skin on the underlying layer.
  3. The method of making sheets or slabs of glass having a thickness of one inch or more, which consists in rolling and casting each sheet in at least three layers formed and fused together progressively, so as to 35 permit each layer to cool partially before the succeeding layer is applied.
  4. The method of making thick homogeneous sheets or slabs of glass which consists in forming each sheet of a plurality of individual layers made progressively and 40 fused together as they are made.
- In testimony whereof, I sign this specification in the presence of two witnesses.
- GEORGE R. MEYERCORD.
- Witnesses:
- HARRY S. GAITHER,  
Wm. F. FRENDENREICH.